

H. PETTIBONE & J. W. ROYER.  
PROCESS OF OXIDIZING AND DRYING OIL CLOTH.  
APPLICATION FILED MAY 3, 1913.

1,176,982.

Patented Mar. 28, 1916.



Fig. 1.



Fig. 2.

Witnesses

J. Milton Gester

Agnes I Stewart

၁၃၄

Inventors

Kawley Pettibone  
Joseph W. Roger  
E. B. Clark

Attorney

# UNITED STATES PATENT OFFICE.

HAWLEY PETTIBONE, OF NEW ROCHELLE, NEW YORK, AND JOSEPH W. ROYER, OF PASSAIC, NEW JERSEY, ASSIGNEES TO THE STANDARD OIL CLOTH COMPANY, OF NEW YORK, N. Y., A CORPORATION OF OHIO.

## PROCESS OF OXIDIZING AND DRYING OIL-CLOTH.

1,176,982.

Specification of Letters Patent.

Patented Mar. 28, 1916.

Application filed May 3, 1913. Serial No. 765,349.

*To all whom it may concern:*

Be it known that we, HAWLEY PETTIBONE, and JOSEPH W. ROYER, citizens of the United States, residing, respectively, at New 5 Rochelle, in the county of Westchester and State of New York, and at Passaic, in the county of Passaic and State of New Jersey, have invented certain new and useful Improvements in Processes of Oxidizing and 10 Drying Oil-Cloth, of which the following is a specification.

This invention relates to treating oil-cloth for imparting a harder, whiter and better finish to the coatings, and reducing the 15 period or time of treatment.

In the manufacture of oil-cloth for table covers, wall covering, and other purposes, the present practice is to apply to the surface a number of coatings, composed principally of china-clay, water, linseed, or other drying oil and a light hydro-carbon, such as naphtha or gasolene, and then hang the coated cloth in folds or festoons in long, narrow closed chambers or cells, provided 20 along the floor with a series of steam pipes or manifolds for effecting the drying operation. These steam pipes, unless the pressure is carried very high, produce only a moderate temperature of about 330 degrees F. in 25 the steam pipe, but result in filling the cell with vapors of water and gasolene, an atmosphere almost devoid of oxygen, which is heavy, sluggish in movement, slow in action and deficient in oxidizing and chemical effect on the oil in the coating. Certain slides 30 are partially opened in the top of the cell, but owing to the heavy character of the vapors the escape thereof is slow, while the loss of heat is considerable, and the drying 35 operation for a cell must extend through a period of five hours or more, so that it is not practicable to make more than two treatments during the working hours of a day in each cell. The effect of the vaporous, sticky 40 atmosphere in the cell is to produce a comparatively soft and unbleached surface on the coating, owing to the lack of oxygen with its hardening and whitening effect upon the linseed oil in the coating. An attempt 45 has been made to remedy these defects by adding a comparatively expensive ingredient,—beeton-white— to the final coating of the cloth, so that the finished surface will be sufficiently white. This adds an objectionable expense to the product and does not hasten or shorten the time required for the drying operation, or aid in oxidizing the oil.

We have found that the expensive steam piping and expensive steam heat supply 55 may be done away with and a much more effective chemical treatment produced—with a saving of 80 per cent., or more, in time, by heating air to a comparatively high temperature, by means of cheap producer gas or by heat produced from other fuel and distributing the air through the treating cell containing the coated cloth. The hot dry air rapidly oxidizes the linseed or other drying oil containing linolein, forming a coherent film of linoxin on the coating, and resulting in bleaching and whitening the same and producing a hard, elastic surface. The hot, expanded air has a great capacity 60 for absorbing moisture and carrying it out of contact with the coated cloth, so that the oxidizing and drying operation can be performed in one to one and a half hours, instead of five, as heretofore required on one class of goods, and two hours instead of 65 twelve hours on another class of goods. In this way, five treatments may be effected in the usual working hours, in each cell, per day, thus permitting continuous treatment 70 in cells of proper dimension.

In addition to reducing the time for drying and treating the coated cloth by eighty per cent., and producing an improved article of manufacture, we also find that by making a producer gas from cheap fuel, we can heat 75 air to a temperature between 400° and 600° F., and with it perform the treating operation above described with a reduction of approximately fifty per cent. in the cost of fuel. Thus, important economy is effected 80 in time of treatment, and in cost of fuel; and an improved article is produced.

The object of our invention, therefore, is 85 to treat coated oil-cloth in a hot, oxidizing, constantly renewed atmosphere, to impart 90

100

to it a harder, whiter and better finished surface; reduce the time of treatment, and effect a saving in the cost of fuel and labor required.

5 The matter constituting our invention will be defined in the claims.

We will now describe more in detail the steps or operations of carrying out our process in connection with the accompanying 10 drawings, in which—

Figure 1 represents a sectional-elevation of an air blower and heater and part of an oil-cloth treating cell. Fig. 2 represents a top plan view of the air blower and heater, 15 partly in section, and part of a treating cell. Fig. 3 represents a transverse section of the treating cell.

In carrying out our process we use a 20 treating chamber or cell A and an air-blowing and heating apparatus B. The cell A is constructed of brick or other suitable material, insulated on the sides, top and bottom with a good non-conductor of heat, and may be made 108 feet long, by 8 feet wide, 25 by 15 feet high, closed at one end, and having door a at the other end for admitting the folds of cloth. We preferably provide a single longitudinal inlet duct H, centrally at the bottom, and having in each side a 30 series of slots or ports h, spaced about as shown throughout the length of the pipe, for discharging numerous streams of hot air outward so that such air may be passed or distributed at numerous points between the 35 suspended folds X of coated cloth. At the top of the cell is placed a longitudinal outlet duct K, having in each side a series of slots or ports k, and extending out through one end of the stack of the cell and connecting 40 with the air-heating furnace, so that vapors may be discharged to the open air.

The air-blowing and heating apparatus B may be of a kind found in the market, and is composed of a combustion chamber or 45 furnace C, having a stack c, provided with a damper c'. A fan D, having a shaft and belt wheel d is driven by an electric, or other motor, E, having on its shaft a belt wheel e, from which is passed a belt e' to the wheel 50 d, for forcing air through the heater and the distributing duct. A four-section, tubular air heater is used, composed of groups or sections G, G<sup>1</sup>, G<sup>2</sup> and G<sup>3</sup> of tubes g, the groups or sections being separated by partition plates in a well known manner, and inclosed in the furnace C. The tubes may be of cast iron, and are connected at their ends in transverse plates, and the groups or sections are connected by the outer end 55 flues F<sup>1</sup>, F<sup>2</sup> and F<sup>3</sup>. A flaring pipe F connects the air blower D with the upper front section G, and the air passes through the tubes g thereof, thence through the tubes of the upper rear section G<sup>1</sup>, thence down 60 through the tubes of the lower rear section

G<sup>2</sup>, and thence through the tubes of the lower front section G<sup>3</sup> to the outlet duct H, which extends through the treating cell and is slotted as above described. A suitable size for the duct H is twenty-four inches wide by 70 twelve inches high in a treating cell of the above described dimensions:

In the division plate between the cold air inlet flue F and the hot air outlet flue H from section G<sup>3</sup> is placed a thermo damper 75 b. In practice this damper may be controlled by a thermostat connected in a known manner with the hot-air flue, so as to maintain the air at a uniform temperature in the discharge flue or duct leading into the treating cell A. This is done by admitting more or less cold air into the outgoing heated air. The temperature of the air may also be maintained at a substantially uniform degree by controlling the flow of gas to the 80 burner in the furnace, either by a thermostatic device, or other means.

A blow-pipe burner M, having a gas-supply pipe m and an air-supply pipe n may be effectively used for heating the air tube sections, and will in practice be connected to the furnace as shown. Producer gas, or a mixture of producer gas and water gas, will, 85 preferably, be delivered at a uniform pressure to the burner.

Near the top of the cell, at each side is fixed a rail L, on which are conveyed in the usual manner the cross-bars l for receiving the folds X of coated oil-cloth, which are spaced and suspended transversely from top to bottom of the chamber so that the numerous streams of air from the ports h may be uniformly distributed between the folds and exert a uniform action on the coatings. The 90 air is heated to a temperature between 400° and 600° F., and distributed in contact with the coated material throughout the treating and drying operation.

The coating preparation is made by mixing together, in suitable proportions, English china clay, water, a drying oil containing linolein, such as linseed oil or China oil, and a light hydro-carbon, as naphtha or gasoline. Other ingredients may be added, and for the last coating beeton-white may be 100 mixed with the other ingredients. The strips of cloth are coated in a well known manner and arranged in folds X on the spaced cross-bars l, so as to be traversed 110 along the longitudinal rails L and thereby fill the cell from end to end with suspended folds or festoons of coated cloth. The cell having been filled and the door a closed the hot air is admitted through the duct H and ports h and distributed at numerous points 115 through and between the folds of material. The hot dry expanded air, having a great capacity for absorbing and carrying moisture, passes up and out through the ports k and outlet duct K to the external air.

Though the air is heated to a temperature above 400° F., and at times to about 600° F., the temperature in the treating cell, owing to the rapid evaporation and circulation, rarely exceeds 200° F., and in no way injures the oil-cloth, even though the high temperature of the air be continued to the end of the operation. The hot and constantly inflowing oxygen acts upon the linolein, rapidly oxidizing the same and forming a film of linoxin, which is hard and coherent, and is appreciably whiter than the surface of goods subjected to steam heat in the ordinary way. The oxidizing and drying operation is completed in one hour instead of five, required by the old method. The cell may therefore be filled, the cloth treated and removed, five times during the usual working hours of a day, effecting a saving of time, or an increase in production amounting approximately to 250 per cent. In other words the process may be made practically continuous. The surface of the treated cloth is entirely free from tackiness, has a hard, coherent protecting surface film, and the goods can be rapidly handled on removal from the cell. We have found that there is especial efficacy in having the oxygen of the air at a high temperature and free as possible from moisture in order that it may act quickly to oxidize the linolein in the oil. We have demonstrated that by this method of using hot air the expense for fuel may be reduced fully one-half as compared with the general method of applying steam heat in coils or manifolds of pipe for heating the cells.

In this process it has been found of the utmost importance that the hot air be distributed with perfect uniformity at numerous points between each pair of pendant folds of cloth and discharged in the same manner through numerous ports substantially opposite the inlet ports, in order to obtain uniform and satisfactory results, in oxidizing and drying the surface of coatings, and to prevent the sticky surfaces from adhering together. There must be no agitating devices in the cell, and no obstruction to cause extra or irregular currents. The hot air is not discharged from inlet ports *h* in strong, irregular currents, but gently and uniformly, so as not to agitate the pendant folds of oil cloth.

Having described our invention, what we claim and desire to secure by Letters Patent, is,—

1. The process of treating and oxidizing oil cloth, having a coating containing linolein, which consists in continuously passing in contact with the coated cloth in a chamber a large volume of fresh oxidizing fluid supplied at a temperature above 300° F. so as to maintain a substantially uniform temperature of about 200° F. in the chamber,—thereby changing the linolein to linoxin

and imparting a whiter, more elastic and better finish to the coating.

2. The process of oxidizing and drying oil cloth, having a coating containing a drying or oxidizing oil and hung in separate folds or festoons in a chamber, which consists in continuously distributing between and in contact with the folds a large volume of air supplied at a temperature between 400° and 600° F., for rapidly oxidizing the oil and forming linoxin with a surface possessing increased hardness, elasticity and whiteness.

3. In the manufacture of oil cloth, having a coating containing linseed oil, the method of treating and drying the same to give it a better surface finish, which consists in rapidly oxidizing the oil to form linoxin by distributing, in contact with the coated cloth, in a chamber, dry air supplied at a temperature between 400 and 600 F., so as to maintain a temperature in the chamber of approximately 200° F. whereby the surface is made harder, and the period of drying is much reduced as compared with the present method of treatment.

4. The process of treating oil-cloth, having a coating containing a drying or oxidizing oil, which consists in heating air to a temperature between 400° and 600° F. and continuously distributing the air at a substantially uniform temperature between and in contact with folds of the cloth in a chamber for constantly bringing fresh oxygen in contact with the coated surface, in a temperature maintained at, or above 200° F. and thereby expediting the oxidizing and drying operation.

5. The process of treating oil-cloth, having a coating containing a drying oil, which consists in distributing hot air between folds of the cloth in a chamber, for constantly bringing fresh oxygen in contact with the surface, and constantly drawing off or discharging the resulting moist or vapor laden air, thereby expediting the oxidizing and drying operation and imparting a better finish to the goods.

6. The process of treating oil-cloth, having a coating containing a drying oil, which consists in distributing hot air at numerous points between folds of the cloth in a chamber, for constantly bringing fresh hot oxygen in contact with the surface, and continuously discharging the resulting moist or vapor laden air at points substantially opposite the inflowing air, for expediting the operation and producing a uniform quality of goods.

7. The process of treating oxidizing and drying oil-cloth, having a coating containing a drying oil, which consists in heating air to a substantially uniform temperature, between 400° and 600° F., distributing the hot air in large volume at numerous points

between folds of the cloth and in contact with its coated surface in a chamber, for removing moisture and rapidly oxidizing the linolein contained in the coating, and continuously drawing off or discharging the moisture-laden air, thereby expediting the operation and imparting to the coating a hard, coherent film of linoxin.

In testimony whereof we affix our signatures in presence of two witnesses.

HAWLEY PETTIBONE.  
JOSEPH W. ROYER.

Witnesses:

HENRY SHELTON,  
W. R. FULLER.